

## 1

3,740,215

## METHOD FOR PRODUCING A HOT WORKED BODY

David L. Burk, Pittsburgh, and Orville W. Reen, Lower Burrell, Pa., assignors to Allegheny Ludlum Industries, Inc., Pittsburgh, Pa.

No Drawing. Filed Aug. 24, 1970, Ser. No. 66,641  
Int. Cl. B22f 7/00

U.S. Cl. 75—208

7 Claims

### ABSTRACT OF THE DISCLOSURE

A method for producing a hot worked body having a low incidence of oxide inclusions. It comprises the steps of consolidating powder comprised of metallic particles into a porous body, substantially sealing the surface of said body by closing surface pores, heating said body, and hot working said body.

The present invention relates to a method of producing a hot worked body having a low incidence of oxide inclusions and more particularly to a method of producing a hot worked body having a low incidence of oxide inclusions from powder comprised of metallic particles.

Today's materials are stronger, last longer, cost less, and are more easily designed and fabricated than the best materials available only a few years ago. They can now be fashioned into smaller parts, larger parts, and more complex shapes than ever before. Largely responsible for creating this advancement in materials technology are modern powder metallurgy processes.

Powder metallurgy processes frequently involve hot working as a means of bringing consolidated metallic bodies to near one hundred percent of reported wrought density. Hot working and heating for hot working must, however, be performed in a non-oxidizing atmosphere to preclude internal oxidation of the bodies, as internal oxidation will limit the attainable density and deleteriously affect properties. Consolidated metallic bodies are particularly susceptible to internal oxidation during hot working as they have an interconnected porosity which accelerates oxygen diffusion.

Various methods have been attempted to preclude internal oxidation during hot working and heating for hot working. One method involved canning of a consolidated powder body under vacuum and hot working of the canned assembly. This process provided adequate protection from oxidation but added extra costs to the hot working operation as it requires a great deal of work in preparing the can and subsequently removing it. A canning procedure is disclosed in U.S. Pat. No. 2,932,882 which issued on Apr. 19, 1960. A second method involved heating in a non-oxidizing atmosphere. This process was disadvantageous insofar as internal oxidation would occur, unless special precautions were taken when the body was transferred from the heating furnace to the hot working apparatus. Another method involved impregnation of the body with a hydrocarbon compound which

## 2

clusions. It comprises the steps of consolidating powder comprised of metallic particles into a porous body, substantially sealing the surface of said body by closing surface pores, heating said body and hot working said body. The step of sealing the surface was found to substantially preclude internal oxidation during both heating and hot working. It provides a dense surface on the body which will resist the penetration of harmful gases at elevated temperatures. In addition, it is advantageous as it rapidly provides a dense surface which is of the same material as the interior, and thus allows the body to be handled in the same manner as a solid bar.

Self-sealing has been disclosed in the past for various reasons, e.g., to improve mechanical strength or to give direction to gas flow within a body. U.S. Pat. Nos. 2,769,709, 3,183,086, and 3,231,430, which respectively issued on Nov. 6, 1956, May 11, 1965, and Jan. 25, 1966, disclose self-sealing. None of these patents, however, disclose or suggest that self-sealing would prevent internal oxidation of a body which is heated and subsequently stretched during hot working.

It is accordingly an object of this invention to provide a method for producing a hot worked body having a low incidence of oxide inclusions from powder comprised of metallic particles.

The method of the present invention comprises the steps of consolidating powder comprised of metallic particles into a porous body, substantially sealing the surface of said body by closing surface pores, heating said body, and hot working said body. Consolidating can involve a cold pressing, hot pressing, or sintering operation or a combination of cold pressing and sintering or hot pressing and sintering. Sintering should be performed in a non-oxidizing atmosphere, e.g., a vacuum, inert gas or reducing gas. Sealing can involve fusion of the surface to fill the pores or mechanical treatment to collapse the pores. Illustrative means of fusing the surface are induction heating, plasma torch fusion, and electron bombardment. Illustrative methods of mechanically sealing the surface are burnishing, machining, and peening. Burnishing is the preferred sealing treatment as it is applicable over a wide range of particle properties and initial densities. Hot working can involve any of the known methods which include extrusion, rolling, swaging, drawing, and forging. It can be performed in air or other oxygen containing atmospheres.

The powder which is to form the hot worked composite can be chosen from a wide spectrum of metals, mixtures of metals, and mixtures of metals and non-metals. Illustrative metals are stainless steel, tool steel, copper, and bronze. Illustrative mixtures are copper-carbon and graphite-bronze.

The following examples are illustrative of the invention.

Predetermined amount of —60 mesh powder from two atomized heats (A+B) were blended to produce a composition which, after sintering, fell within the chemical specification of A.I.S.I. Type 304 stainless steel. The blend ratio and chemical composition of the constituent heats are listed below in Table I.

TABLE I

| Heat   | Percentage<br>of heat in<br>blend | Composition of heat |      |       |       |      |       |       |      |
|--------|-----------------------------------|---------------------|------|-------|-------|------|-------|-------|------|
|        |                                   | C                   | Mn   | P     | S     | Si   | Cr    | Ni    | Fe   |
| A----- | 26.0                              | 0.44                | 0.29 | 0.018 | 0.010 | 2.06 | 18.19 | 12.37 | Bal. |
| B----- | 74.0                              | 0.009               | 0.18 | 0.003 | 0.006 | 1.75 | 17.92 | 12.40 | Bal. |

evolves a protective vapor during heating. This process is not totally satisfactory as it employs a material different from the metal of the body. It is disclosed in U.S. Pat. No. 3,152,893 which issued on Oct. 13, 1964.

The present invention provides a method for producing a hot worked body having a low incidence of oxide in-

70  
Three bodies were prepared from the blend. Loose powder was poured, tamped, and vibrated into rubber isostatic consolidating bags measuring approximately 3.2 inches in diameter by 9 inches long, hydrostatically consolidated at pressures of 20, 25, and 30,000 p.s.i. and vacuum sintered for six hours at 2400° F. The bodies

were about 2.75 inches in diameter and about 7 inches long.

The bodies were prepared for extrusion by drilling a  $\frac{7}{8}$  inch hole through their centers and by machining the outer diameters to 2.62 inches. Both the inner and outer diameters as well as the ends and corners were then burnished. The burnished outer diameter was 2.60 inches. Extrusion was subsequently carried out with the bodies at a temperature of from 2000 to 2200° F. The bodies were heated in air with an induction heating coil.

The extruded bodies were examined metallographically for the presence of internal oxidation. The examination revealed that internal oxidation was not present. Burnishing provided a dense surface on the bodies which resisted the penetration of harmful gases during heating and hot working and, thereby, precluded internal oxidation.

From the above paragraphs it will be apparent to those skilled in the art that the novel principles of the invention disclosed herein in connection with specific examples thereof will suggest various other modifications and applications of the same. It is accordingly desired that in construing the breadth of the appended claims they should not be limited to the specific examples described herein.

We claim:

1. A method of producing a hot worked body having a low incidence of oxide inclusions from powder comprised of metallic particles, which comprises the steps of: consolidating powder comprised of metallic particles into a porous body; substantially sealing the surface of said body by closing surface pores; heating said body in an oxidizing atmosphere; and hot working said body in an oxidizing atmosphere, said sealing of said surface substantially precluding internal oxidation during said heating and said hot

working by providing a dense surface which resists the penetration of harmful gas at elevated temperatures.

2. A method according to claim 1 wherein the surface is substantially sealed by fusing the surface to fill the pores.

3. A method according to claim 1 wherein the surface is substantially sealed by mechanically treating the surface to collapse the pores.

4. A method according to claim 3 wherein said surface is mechanically treated by burnishing said surface.

5. A method according to claim 1 wherein said powder is consolidated by cold pressing powder and sintering said pressed powder in a non-oxidizing atmosphere and wherein said body is hot worked by extruding said body.

6. A method according to claim 1 wherein said body is heated in air.

7. A method according to claim 1 wherein said metallic particles are steel particles.

#### References Cited

##### UNITED STATES PATENTS

|           |         |              |       |          |
|-----------|---------|--------------|-------|----------|
| 2,215,723 | 9/1940  | Jones        | ----- | 75—208 R |
| 2,220,641 | 11/1940 | Davis        | ----- | 75—200 X |
| 2,839,397 | 6/1958  | Cavanaugh    | ----- | 75—222   |
| 2,997,777 | 8/1961  | Davies       | ----- | 29—182   |
| 3,183,086 | 5/1965  | Kurtz et al. | ----- | 75—208 R |

CARL D. QUARFORTH, Primary Examiner

R. E. SCHAFER, Assistant Examiner

U.S. Cl. X.R.

29—182.2, 420.5; 75—214